

V. B. BROWNE,  
MANUFACTURE OF STEEL SHEETS.  
APPLICATION FILED JUNE 9, 1919.

1,340,149.

Patented May 18, 1920.



WITNESSES

J. Harold Bradley.

INVENTOR

Vern B. Browne  
J. De S. Brown  
a.m.

# UNITED STATES PATENT OFFICE.

VERE B. BROWNE, OF TARENTUM, PENNSYLVANIA.

## MANUFACTURE OF STEEL SHEETS.

1,340,149.

Specification of Letters Patent. Patented May 18, 1920.

Application filed June 9, 1919. Serial No. 302,913.

To all whom it may concern:

Be it known that I, VERE B. BROWNE, a citizen of the United States, and a resident of Tarentum, in the county of Allegheny and State of Pennsylvania, have made a new and useful Invention in the Manufacture of Steel Sheets, of which the following is a specification.

This invention relates to the manufacture of steel sheets of extreme thinness.

For a number of years attempts have been made by hot rolling methods to manufacture steel sheets of extreme thinness, that is sheets of 2/1000 of an inch and less. In certain of the arts there is a growing demand for such steel sheets and so far as I know no one, in this country at least, has been able to produce the same commercially.

In certain branches of the electrical art there is a demand for such sheets made from silicon steel and there is also a demand for sheets made from mild steel.

An object of this invention is to provide a method whereby steel of any desired analysis may be commercially rolled into sheets of 2/1000 of an inch and less in thickness.

This, as well as other objects which will readily appear to those skilled in the art of making steel sheets, I attain in the method hereinafter set forth.

In rolling these extremely thin sheets under standard sheet or tin mill practice to less than 6/1000 of an inch in thickness it is impossible to separate the sheets without tearing them.

The drawing is a sectional elevation showing a pack formed according to a preferred form of my method.

My method consists in utilizing any standard sheet or tin mill practice to produce sheets of the desired analysis and approximately 6/1000 of an inch in thickness. Such sheets are then taken separately and placed between relatively heavy sheets of steel of different general characteristics; that is a pack of any desired number of sheets is built up of sheets of the special steel alternating with relatively heavy sheets of steel having different general characteristics and the built-up pack is then rolled to length thus reducing the special or inner sheets to the desired thinness.

I have found that a desirable method is to bring the relatively heavy sheets to rolling

temperature and to alternate these with 55 sheets of the special steel in a cold state. The special steel sheets take up sufficient heat from the relatively heavy hot sheets for rolling. If desired this built-up pack may consist of but three sheets, one relatively 60 thin sheet in a cold state of the special steel sandwiched between two relatively thick sheets of dissimilar steel which have been brought to rolling temperature. Instead of placing the special steel sheets in a cold state 65 between relatively heavy sheets brought to rolling temperature the pack which may consist of any suitable number of sheets may be built-up and then brought to rolling temperature (preferably a low rolling temperature). These built-up packs may be worked under any of the standard mill methods and if desired may be doubled or otherwise manifolded according to any of the approved methods. If doubled the pack 70 after being rolled to length will be sheared and opened in the usual way.

On account of having the special sheets arranged alternately with heavier sheets of dissimilar steel the separation of the finished sheets is readily affected since the dissimilar sheets under the rolling will not weld with the special sheets, neither will the surface tension or other forces tending to hold the sheets together be great enough to 85 cause the sheets to tear during separation.

If the special sheets are silicon steel the sheets with which they alternate may be mild steel and if the special sheets are mild steel the sheets with which they alternate 90 may be silicon steel. It is always necessary to see that the sheets on the outside of the pack are the relatively heavy sheets.

Having thus described my invention what I claim is—

1. The method of rolling extremely thin sheets of steel, which consists in producing a relatively thin sheet, in sandwiching said sheet between sheets of steel of heavier gage and different general characteristics and 100 then in hot rolling the sandwiched sheets to such length as to give the desired thickness to the inner sheet.

2. The method of rolling extremely thin sheets of silicon steel, which consists in producing a relatively thin sheet, in sandwiching said sheet between two sheets of steel of heavier gage and different general char- 105

acteristics and then in hot rolling the sandwiched sheets to such length as to give the desired thickness to the inner sheet.

3. The method of rolling an extremely thin sheet of metal, which consists in placing a relatively thin sheet of such metal in a cold state between two heavier sheets of metal having dissimilar characteristics and brought to a rolling temperature and then 10 in reducing the gage of the three-ply pack.

4. The method of rolling sheets of steel of 2/1000 of an inch or less in thickness, which consists in producing a sheet no thicker than 14/1000 of an inch, in sandwiching said sheet between two sheets of steel of heavier gage and then in hot rolling the sandwiched sheets to such length as will give the desired thickness to the inner sheet.

5. The method of rolling sheets of steel of 2/1000 of an inch or less in thickness, which consists in producing a sheet no thicker than 14/1000 of an inch, in sandwiching said sheet while cold between two hot sheets of steel of heavier gage and having different characteristics therefrom and then in reducing the sandwiched sheets to such length as will give the desired thickness to the inner sheet.

6. The method of rolling extremely thin sheets of silicon steel, which consists in producing a relatively thin sheet, in sandwiching said sheet while cold between two heated sheets of steel having different characteristics and of heavier gage and then in rolling the sandwiched sheets to such length as to give the desired thickness to the inner sheet.

7. The method of rolling extremely thin sheets of steel, which consists in alternating cold relatively thin sheets with heavier sheets of steel of different characteristics raised to rolling temperature, and then in rolling the multi-ply pack to produce sheets of the desired gage.

45 8. The method of rolling extremely thin sheets of steel, which consists in alternating cold relatively thin sheets with heavier sheets of dissimilar steel raised to rolling temperature, and then in rolling the multi-ply pack 50 to produce sheets of the desired gage.

9. The method of rolling an extremely

thin sheet of metal, which consists in placing a relatively thin sheet of such metal in a cold state between two heavier sheets of other metal in a heated state and then in 55 reducing the gage of the three-ply pack.

10. The method of rolling an extremely thin sheet of metal, which consists in placing a relatively thin sheet of such metal in a cold state between two heavier sheets of 60 metal having dissimilar characteristics and in a heated state and then in reducing the gage of the three-ply pack.

11. The method of rolling sheets of steel of 2/1000 of an inch or less in thickness, 65 which consists in producing a sheet no thicker than 14/1000 of an inch, in sandwiching said sheet while cold between two heated sheets of steel having different characteristics and of heavier gage then in rolling the sandwiched sheets to such length as 70 will give the desired thickness to the inner sheet.

12. The method of hot rolling a sheet of metal of less than 6/1000 of an inch in thickness, which consists in producing a relatively thin sheet, placing said sheet between two materially heavier sheets of metal having dissimilar characteristics and then in reducing the gage of the multiple pack by 75 hot rolling, substantially as described.

13. The method of hot rolling a sheet of steel to 3/1000 of an inch or less in thickness, which consists in producing a relatively thin sheet, placing said sheet between 85 two metal sheets of materially heavier gage and different characteristics raised to rolling temperature and then in hot rolling the multiple pack, substantially as described.

14. A hot rolled sheet of silicon steel 90 under 6/1000 of an inch in thickness.

15. A hot rolled sheet of silicon steel 3/1000 of an inch or less in thickness.

16. A hot rolled sheet of steel less than 6/1000 of an inch in thickness. 95

17. A hot rolled sheet of steel 3/1000 of an inch or less in thickness.

18. A rolled sheet of silicon steel 2/1000 of an inch or less in thickness.

In witness whereof, I have hereunto subscribed my name this 5th day of June, 1919.

VERE B. BROWNE.